

Jan. 8, 1929.

1,698,623

R. B. DALE

ROTARY CASTING

Filed Dec. 23, 1925

3 Sheets-Sheet 1



Inventor:  
R. Burdette Dale  
per Augustus M. Stenay  
Attorney.

Jan. 8, 1929.

1,698,623

R. B. DALE

ROTARY CASTING

Filed Dec. 23, 1925

3 Sheets-Sheet 2



Inventor:  
R. Burdette Dale  
per Augustus M. Henry  
Attorney.

Jan. 8, 1929.

1,698,623

R. B. DALE

ROTARY CASTING

Filed Dec. 23, 1925

3 Sheets-Sheet 3

Fig. 5.



R. Burdette Dale  
Inventor

By his Attorney  
Augustus M. Henry

## UNITED STATES PATENT OFFICE.

ROBERT BURDETTE DALE, OF JAMAICA, NEW YORK, ASSIGNOR TO WILLIAM W. WEITLING, OF COLLEGE POINT, LONG ISLAND, NEW YORK.

## ROTARY CASTING.

Application filed December 23, 1925. Serial No. 77,188.

This invention relates to casting; is particularly useful in rotary casting; and is applicable, in connection with rotary or non-rotary molds to the casting of the ferrous metals, as iron and even steel.

The general advantages of the present invention may perhaps be most clearly indicated by a short discussion at this point of the importance of the invention in making ferrous castings in rotary molds.

In the casting of ferrous metal articles such as iron or steel pipe, by the rotary or centrifugal method, there are two main objects which must always be kept in mind, 15 where the mold is a permanent one in the sense that a considerable number of castings are to be made without injuring the mold or its lining. Such a permanent mold must be used if the rotary method of manufacture is 20 to be rapid and economical enough to warrant its installation. As far as I am aware, all rotary casting methods heretofore proposed and now operating successfully or apparently capable of such operation, employ 25 a permanent mold which is of metal.

Of the two main objects above referred to, which must always be kept in mind, one is to insure that the ferrous casting shall not be chilled so that an annealing or other heat 30 treating thereof is required after the casting has been removed from the mold. The other main object to be kept in mind is to have present as a feature of the process a method of or a means for exercising a supervision 35 and control over the temperature of the mold, not only to provide a ferrous casting unchilled as above, but also to minimize abruptness of mold temperature changes, particularly if the mold be a metal mold, 40 during the casting operation and between successive casting operations.

Such a method and means as that last described is disclosed in my copending application Serial No. 749,476, filed November 12, 45 1924; where I propose the use of a metal structure including an inner mold proper or shaping member and an outer tubular member spaced from the mold proper to provide an annular chamber for contained mercury vapor. According to this arrangement, the pressure of the vapor jacket is raised and lowered at intervals during the casting operation and between successive casting operations, thereby to raise and lower the tempera-

ture of the mold and the charge being cast 55 therein precisely as prevised; advantage being taken of the fact that a mercury-vapor pressure change causes an immediate and corresponding change in temperature, yet with high-temperature conditions always accompanied by relatively low-pressure conditions as compared with steam. In said co-pending application, there is disclosed a plurality of rotary casting machines interconnected as to their annular chambers 60 by way of a hermetically closed circulatory system for the mercury vapor to serve several or all the casting machines simultaneously but preferably differentially; so that one or more of such chambers may 65 have the pressure of their vapor blankets increased wholly or partly as the result of decreasing the pressures of the vapor blankets of another or other machines. By such an arrangement fairly rapid production is 70 possible from each of the machines; it being clear that while one machine is receiving its charge of molten metal, another machine is spinning its previously received charge into shape and into set, another machine is spinning to further set its casting, another machine is being stopped rotating preparatory to removing its casting, another machine has stopped rotating and is having its casting removed, another machine is being inspected 75 after the removal of its casting and being otherwise made ready for spinning for receiving another charge, and so on, depending on the number of machines in the set or battery of each production unit. According 80 to said system, also, a mercury boiler or boilers are incorporated in the closed system, for replenishing the vapor supply should production be halted for an unusually long time for any reason; and the system 85 also includes one or more condensers preferably forming parts of steam generators or other heat interchangers or economizers for usefully abstracting the large number of excess B. t. u.'s developed over a prolonged 90 casting period during which castings are made at a fairly rapid rate.

The present invention aims to provide certain improvements in regard to a method and apparatus capable of being carried out by 105 and embodied in a single casting machine such as that just described or an equivalent, or in a system such as that just described or

- an equivalent. These improvements have the particular object of making the process of said copending application a truly commercial one, and not only that but a highly economical and profitable one, because of greater ease of supervision and control of the rate of congelation of a casting, and because of greater speed in turning out each casting as well as a given run of castings.
- 10 To these ends, the present invention aims to provide, among other things, first, a means of and apparatus for spraying or otherwise suitably introducing liquid mercury into the vapor chamber of a casting machine, as and when required, and second, a means of and apparatus for positively discharging from said chamber, and collecting for such discharge if necessary, liquid mercury in the chamber, as and when required.
- 15 20 It should be explained in this connection that introducing liquid mercury into the chamber increases immensely the rate of cooling of the casting, due to the heat absorbed by the liquid mercury when the same is vaporized by contact with the walls of the chamber.
- 25 As the present invention is preferably carried out, the same provides a method of and apparatus for (1) utilizing a predetermined vapor blanket pressure to hold the mold temperature high enough, at or up to the introduction of a molten charge, to permit the molten metal to be held molten over a sufficient length of time to insure that the charge will properly distribute itself in the mold, however unevenly such charge be delivered to the mold; (2) thereafter utilizing another predetermined pressure to permit the casting to set at as rapid a rate as possible and yet with that degree of slowness of set required to insure that the third shrinkage of the casting shall occur before the precipitation of cementite, or otherwise to insure that the casting will so slowly cool down to a critical point that, however rapidly thereafter the casting is cooled, the same will not after removal from the mold be so much chilled as to require a subsequent annealing or heat treating; (3) thereafter utilizing another predetermined pressure of the vapor and, in combination therewith, an injection of liquid mercury, to cool the casting beyond said critical point at a very rapid rate, thereby very quickly to impart to the casting such surface freeze or other rigidity that it may safely be removed from the mold; and (4) thereafter utilizing another predetermined pressure of the vapor to raise the temperature of the mold to that high temperature referred to under (1), if another casting is to be made during the run; while (5) collecting, and discharging practically as soon as collected from the annular chamber, all liquid mercury injected in excess of that evaporized

according to (3), and all liquid mercury condensed or otherwise accumulated in the chamber.

The invention will be more clearly understood from the following description, when taken in connection with the accompanying drawings, showing one possible apparatus adapted to constitute a structural embodiment of the invention and one facilitative of a carrying out the method of the invention; it being understood, however, that all matter shown in the drawings, and all matter herein contained except in the appended claims, is merely illustrative and not to be taken in a limiting sense. In other words, said claims define the scope of protection contemplated; and said claims, of course are to be given full range of equivalents.

In the drawings,

Fig. 1 shows a pipe casting machine in side elevation, certain of the hidden parts being shown in broken lines;

Fig. 2 is an enlarged vertical axial section of the bell end of the mold;

Fig. 3 is a transverse section, taken on the line 3—3 of Fig. 1;

Fig. 4 is a vertical axial section of the opposite end of the mold, and

Fig. 5 is an almost completely self-explanatory diagram relative to the casting of a cast iron pipe.

The machine as shown in Fig. 1 includes a rotary structure including an outer casing 5. This structure is journaled at opposite ends in frames 6, and carries a center collar-structure 7 forming part of the rotating drive. At 8 is indicated a core carrier, rotary on a charge delivering spout 9 (so that the core carrier may rotate with the mold, relative to the spout). The spout is fed by hopper 10 on a pedestal 11 vertically pivoted on a wheel truck 12; so that during a casting operation, with the parts as shown, and assuming it is desired to cast a belled pipe, the core is properly in the mold to make such bell therearound, and so that, after a casting operation, the truck may be moved on its wheels sufficiently to the left to permit the spout and core carrier to be cleared from the mold, by swinging the pedestal on its pivot.

Referring now to Figs. 2, 3 and 4, it will be seen that said outer casing 5, carrying at opposite ends internal collar-structure 13 and 14, is neither the double-walled mold proper 15—15<sup>a</sup> nor the outer tubular member 16 surrounding the annular vapor chamber 17, but is a carrier for the parts last mentioned by way of such collar-structures and also a housing means for a mass of suitable heat insulating material 18.

In order hermetically to close the annular chamber 17 at the bell end of the machine, the outer wall 15 of the mold proper is outwardly peripherally flanged as shown, and

welded to the tubular member 16 as indicated at 19 in Fig. 2; and, as shown in Fig. 4, the opposite end of the mold is closed by a circular plate 20 to which an inwardly bent peripheral portion of the wall 15 of the mold proper is welded as indicated at 21.

The tubular member 16, which at the bell end of the machine is secured to collar-structure 13, is conically reduced beyond the 10 other end of the mold proper and thence extends to where it is secured to collar structure 14 at the opposite end of the machine. Beyond this point, an integral prolongation 16' of the tubular member rotates in a journal-box 22<sup>a</sup> formed in a frame 22.

As will be seen clearly from Figs. 2 and 4, the tubular member 16 is hollow from end to end, to form the annular chamber 17 as required and to permit mercury vapor to be 20 admitted or to be drawn off, and to be changed in pressure and hence in temperature, by way of a single combined inlet and outlet at the free end of the prolongation 16' of the tubular member 16, and by 25 way of a suitable valve-served passage 23 formed in frame 22.

Beyond this passage 23, the frame 22 carries a journal-box 24 coaxial with the journal-box 22<sup>a</sup>, for receiving an end of 30 a main feed tube 25 terminating at its opposite end in a conical manifold 26 serving a plurality of spiral spray tubes 27 for liquid mercury. Main tube 25, at its open end removed from said manifold, is in communication with a suitable valve-served passage 28 in frame 22.

Each of these spiral spray tubes is supported and rigidified by being disposed, and secured if desired, against the advancing side 40 (note the arrow of Fig. 3, indicating the direction of the rotation of the mold) of one of four spiral blades 29. These blades are suitably secured, as by welding, to the inner surface of tubular member 16, from well 45 beyond the spacing collar 30 at the bell end of the machine as shown best in Fig. 2, to the outer or free end of the prolongation of 16' of the tubular member 16. Referring in this connection to Fig. 4, said blades of 50 course are shaped in the vicinity of the conically reduced portion of the tubular member 16 and in the vicinity of the conical manifold 26 and the main tube 29<sup>a</sup>, to conform thereto, and are edge welded to the rounded 55 surfaces thereof.

The mold proper 15—15<sup>a</sup> is of course centered in the tubular member 16 at the bell end of the machine by the means already described and including the welding 19 shown in Fig. 2. At the opposite end of 60 the machine, the mold proper may be further secured and centered by incorporating such an arrangement as the collar-structure indicated at 31, which will be cut out at 65 intervals all around in order to permit pas-

sage of the blades and the spray tubes and also to provide mercury vapor ports.

Said blades constitute in the machine illustrated, means for collecting and discharging liquid mercury in the annular 70 chamber 17. Obviously, without such blades or some equivalent means, the faster the mold is rotated, the more securely will mercury in said chamber and particularly 75 in the outlying portions thereof opposite the bell end of the mold, become trapped by centrifugal force, against removal by way of the bore of prolongation 16' of the tubular structure 16; whereas, with such blades present, and arranged as shown, and the 80 mold rotating as shown in Fig. 3, as soon as the mold is rotated at any speed below a permissible maximum, such liquid mercury will be collected, transported to and discharged from said bore. Hence, to remove 85 liquid mercury, and to remove the same by discharging it into vapor passage 23, thus to return the liquid mercury preferably by way of a liquid trap, to the closed system 90 for use therein as explained in the copending application aforesaid, it is only necessary to start rotating the mold at that speed whereat centrifugal force will not be so effective on the liquid as to interfere with the gravity 95 action thereon. This gravity action is that which causes the liquid actually to "puddle", despite the rotation of the mold, in the bottom of annular chamber 17, there to be picked up by the advancing side of a blade 29, and thereafter, consequently, to flow 100 downwardly along said blade toward and through the bore in prolongation 16' of tubular structure 16; as contrasted with the situation which would otherwise prevail 105 when the mold would have to be stopped rotating and dismantled or up-ended in order to remove the liquid mercury.

From the explanations hereinabove, it will be seen that, during rotation of the mold, both gravity and centrifugal force alternately act, in an ideal way, to accomplish the desired result, which is to prevent clearing, and to clear, the annular chamber 17 of liquid mercury, at certain appropriate intervals in the cycle of the making of a single casting or a run of castings. Thus, whenever the mold-temperature is to be affected by the removal of liquid mercury, whether the latter be that injected as such or liquid previously condensed from mercury vapor, the mold is always rotating, and what is quite as important, rotating below that speed whereat the blades or vanes 29 will function positively to discharge the liquid mercury. In this connection, see the diagram of Fig. 5. First, however, it should be made clear that this diagram is merely illustrative of the general principle, and fortuitous circumstances, involved; that, as indicated by one of the legends in said dia- 115 120 125 130 135

gram, the showing assumes the making of cast iron pipe; and that, in said diagram, no attempt has been made to include or otherwise indicate time intervals or relations by 5 lengths of various portions of the curves or by relations between such curves or their portions. In this diagram, the legend "L. M.—Egress speed", the L. M. standing for "liquid mercury", means the maximum permissible speed for vane-ejections of liquid mercury; and consequently the range of 10 mold speeds whereat such ejection will take place, is indicated at V. The broken lines forming part of the arrows and located before 15 the arrow-heads, at the three places shown on the diagram, indicate that the conclusions of the operations described are, individually, particularly susceptible of variation under different conditions. In a cycle 20 including a run of castings, the two main curves will repeat on themselves, as by imagining the point C', each time the point C is reached, to become projected to the location of the point C. It being finally noted 25 that the legend "Critical point" refers to the critical point hereinabove mentioned, it is believed that further explanation of the diagram is unnecessary.

Obviously, the present invention is not to 30 be limited to the casting of ferrous metals, or indeed the casting of any metals; or to casting in centrifugal or rotary molds. Nor is the invention to be limited to a utilization necessarily involving a permanent mold 35 which is of metal, or even a permanent mold of any kind. Further, the invention is not to be limited to the casting of elongate articles of circular cross section such as pipe, or even disk-like articles such as car wheels. 40 Again, the invention is not necessarily to be limited to mercury vapor and liquid mercury if another vapor and another liquid, whether or not such vapor be merely said liquid in another form, be found susceptible 45 of employment according to the broad principles of the invention. In other words it is emphasized, again, that the pending claims are to be looked to solely, for the definition of the real fundamentals of the 50 present invention; all other things shown and described herein being merely illustrative of a preferred mode of carrying out the invention as now understood.

I claim:

55 1. In the art of rotary casting, the method of affecting the rate at which the mold and mold-coadjuvant parts of a casting machine absorb heat from a material being cast in the mold, which involves bringing a metallic liquid having a vaporization temperature considerably lower than zinc, into contact 60 with one of such heat-absorptive parts.

2. In the art of rotary casting, the method of affecting the rate at which the mold and 65 mold-coadjuvant parts of a casting machine

absorb heat from a material being cast in the mold, which involves directing a liquid metal into heat-absorptive relation to the mold.

3. In the art of rotary casting, the method of affecting the rate at which the mold and mold-coadjuvant parts of a casting machine absorb heat from a material being cast in the mold, which involves alternately bringing a heat-absorptive liquid into heat-absorptive relation to one of such heat-absorptive parts, and removing said liquid from said relation. 75

4. In the art of rotary casting, the method of affecting the rate at which the mold and mold-coadjuvant parts of a casting machine absorb heat from a material being cast in the mold, which involves spraying a liquid against one of such heat-absorptive parts, and utilizing centrifugal force to distribute 80 the sprayed liquid. 85

5. In the art of rotary casting, the method of affecting the rate at which the mold absorbs heat from a material being cast therein, which involves bringing a non-oleaginous liquid into heat-exchanging relation with the mold, said liquid being vaporizable at a higher temperature than water but at a lower temperature than zinc. 90

6. In the art of rotary casting, the method of affecting the rate at which the mold absorbs heat from a material being cast therein, which involves bringing a non-aqueous and non-oleaginous liquid and a liquid free of considerable quantities of lead, zinc or tin, 100 into heat-interchanging relation with the mold. 105

7. In the art of rotary casting, the method of affecting the rate at which the mold and mold-coadjuvant parts of a casting machine absorb heat from a material being cast in the mold, which involves spraying a liquid into heat-exchanging relation to one of such heat absorptive parts in a plurality of jets, in non-straight-line relation. 110

8. In the art of rotary casting, the method of affecting the rate at which the mold and mold-coadjuvant parts of a casting machine absorb heat from a material being cast in the mold, which involves spraying a liquid into heat-exchanging relation to one of such heat-absorptive parts in a plurality of jets circumferentially spaced. 115

9. In the art of rotary casting, the method of affecting the rate at which the mold and mold-coadjuvant parts of a casting machine absorb heat from a material being cast in the mold, which involves spraying a liquid into heat-exchanging relation to one of such heat-absorptive parts in a plurality of jets arranged in a plurality of substantially parallel lines. 120

10. In the art of rotary casting, the method of affecting the rate at which the mold and mold-coadjuvant parts of a cast- 130

ing machine absorb heat from a material being cast in the mold, which involves spraying a liquid into heat-exchanging relation to one of such heat-absorptive parts in a 5 plurality of jets arranged in a substantially spiral line.

11. In the art of rotary casting, the method of affecting the rate at which the mold absorbs heat, which involves alternately predeterminedly bringing into heat-exchanging relation with the mold a liquid, and a vapor.

12. In the art of rotary casting, the method of affecting the rate at which the 15 mold absorbs heat, which involves alternately predeterminedly bringing into heat-exchanging relation with the mold, a vapor under a given pressure, a liquid, and a vapor under a different pressure from that first 20 mentioned.

13. In the art of rotary casting, the method of affecting the rate at which the mold absorbs heat, which involves alternately predeterminedly bringing into heat-ex- 25 changing relation with the mold a liquid, and a vapor under a predetermined pressure.

14. In the art of rotary casting, the method of affecting the rate at which the mold absorbs heat, which involves main- 30 taining a vapor in heat-exchanging relation with the mold, at intervals bringing a liquid into heat-exchanging coaction with said vapor relative to the mold, and at intervals removing a part of said liquid from 35 such coaction.

15. In the art of rotary casting, the method of using a liquid, and a vapor in confinement, for coacting to affect the rate 40 of heat-absorption of the mold, which involves employing centrifugal force to dis- tribute said liquid relative to the vapor.

16. In the art of rotary casting, the method of using a liquid, and a vapor in confinement, for coacting to affect the rate 45 of heat-absorption of the mold, which involves employing centrifugal force to dis- tribute said liquid relative to the vapor and gravity to collect said liquid for discharge from said confinement.

50 17. In the art of rotary casting, the method of using a liquid, and a vapor in confinement, for coacting to affect the rate of heat-absorption of the mold, which involves employing mold-rotation to discharge 55 said liquid from such confinement.

18. In the art of rotary casting, the method of using a liquid, and a vapor in confinement, for coacting to affect the rate of heat-absorption of the mold, which involves employing mold-rotation to segregate 60 said liquid from the vapor, while confining the liquid and the vapor in predetermined adjacency to the mold, and also positively to discharge the liquid from said 65 confinement.

19. In the art of rotary casting, the method of using a medium in vapor form to affect the rate of heat-absorption of the mold, such liquid becoming liquid at a certain temperature; which involves confining such 70 vapor in predetermined adjacency to the mold and utilizing mold-rotation to remove from said adjacency a part of the medium becoming liquid while in such adjacency.

20. In rotary casting, the method of af- 75 fecting the rate of congelation of a casting, which involves subjecting such casting to heat-exchanging relation with mercury vapor, and simultaneously to similar relation with a liquid.

21. In rotary casting, the method of af- 80 fecting the rate of congelation of a casting, which involves subjecting such casting to heat-exchanging relation with a vapor, and simultaneously to similar relation with 85 liquid mercury.

22. In rotary casting, the method of af- 90 ffecting the rate of congelation of a casting, which involves subjecting such casting to heat-exchanging relation with mercury va- por, and simultaneously to similar relation with liquid mercury additional to any liquid mercury then in such relation as the result of condensation from mercury vapor previously in such relation.

23. In rotary casting, the method of af- 95 ffecting the rate of congelation of a casting, which involves subjecting such casting to heat-exchanging relation with mercury va- por, and simultaneously to similar relation 100 with liquid mercury, and then to similar relation with such vapor and a less amount of such liquid.

24. In the art of rotary casting, the meth- 105 od of affecting the rate at which the mold absorbs heat from a material being cast therein, which involves providing a jacketed mold, and spraying a liquid into the jacket during setting in the mold of the ma- terial being cast.

25. In the art of casting, the method of 110 affecting the rate at which the mold absorbs heat from a material being cast therein, which involves providing a jacketed mold, and spraying a liquid into the jacket during 115 setting in the mold of the material being cast.

26. In the art of casting, the method of 120 affecting the rate at which the mold absorbs heat from a material being cast therein, which involves bringing a non-aqueous and non-oleaginous liquid and a liquid free of considerable quantities of lead, zinc or tin, into heat-interchanging relation with the mold.

27. In the art of casting, the method of 125 affecting the rate at which the mold and mold-coadjuvant parts of a casting machine absorb heat from a material being cast in the mold, which involves spraying a liquid 130

into heat-exchanging relation to one of such heat-absorptive parts in a plurality of jets in non-straight-line relation.

28. In the art of casting, the method of affecting the rate at which the mold absorbs heat, which involves alternately predeterminedly bringing into heat-exchanging relation with the mold a liquid, and a vapor.

29. In the art of casting, the method of affecting the rate at which the mold absorbs heat, which involves alternately predeterminedly bringing into heat-exchanging relation with the mold, a vapor under a given pressure, a liquid, and a vapor under a different pressure from that first mentioned.

30. In the art of casting, the method of affecting the rate at which the mold absorbs heat, which involves alternately predeterminedly bringing into heat-exchanging relation with the mold a liquid, and a vapor under a predetermined pressure.

31. In the art of casting, the method of affecting the rate at which the mold absorbs heat, which involves maintaining a vapor in heat-exchanging relation with the mold, at intervals, bringing a liquid into heat-exchanging coaction with said vapor relative to the mold, and at intervals removing a part of said liquid from such coaction.

32. In casting, the method of affecting the rate of congelation of a casting, which involves subjecting such casting to heat-exchanging relation with mercury vapor, and simultaneously to similar relation with a liquid.

33. In casting, the method of affecting the rate of congelation of a casting, which involves subjecting such casting to heat-exchanging relation with a vapor, and simultaneously to similar relation with liquid mercury.

34. In casting, the method of affecting the rate of congelation of a casting, which involves subjecting such casting to heat-exchanging relation with mercury vapor, and simultaneously to similar relation with liquid mercury additional to any liquid mercury then in such relation as the result of condensation from mercury vapor previously in such relation.

35. In casting, the method of affecting the rate of congelation of a casting, which involves subjecting such casting to heat-exchanging relation with mercury vapor, and simultaneously to similar relation with liquid mercury, and then to similar relation with such vapor and a less amount of such liquid.

36. In the art of rotary casting of metals, a method of affecting the rate at which the mold absorbs heat, which involves alternately bringing into heat-exchanging relation with the mold during solidification of the casting in the mold, a liquid, and a vapor.

37. A method according to claim 36, char-

acterized by bringing into such heat-exchanging relation with the mold a vapor under a given pressure, a liquid, and a vapor under another pressure.

38. A method according to claim 36, characterized by causing the vapor and the liquid to coact heat-exchangingly, and removing some or all of said liquid from such coaction, said vapor being the vapor of a liquid existent as a vapor at a high temperature and low pressure as compared with steam.

39. A method according to claim 36, wherein the liquid and the vapor are used in confinement, for coacting to affect the rate of heat absorption of the mold, and thereby with the rate of congelation of a casting in the mold.

40. A method according to claim 36, wherein centrifugal force is employed to distribute said liquid relative to the vapor and gravity to collect said liquid for discharge from said confinement.

41. A method according to claim 36, characterized by employing mold-rotation to segregate said liquid from the vapor and to positively discharge the liquid from such relation.

42. A method according to claim 36, wherein said liquid is a metal.

43. A method according to claim 36, wherein said liquid is liquid mercury.

44. A method according to claim 36, wherein said vapor is mercury vapor.

45. A method according to claim 36, wherein said liquid is liquid mercury and said vapor is mercury vapor, and wherein said liquid mercury is deliberately added as an addition to liquid mercury then present as the result of condensation.

46. A rotary metal casting apparatus having a rotary mold and a vapor chamber associated therewith in heat exchanging relation thereto in combination with means for at will admitting vapor to said chamber, and means for spraying liquid into said chamber.

47. A rotary casting apparatus according to claim 46, including means for moving any such liquid in the chamber axially of the mold.

48. A rotary casting apparatus according to claim 46, including a spiral blade arranged in said chamber and adapted to move said liquid axially toward an outlet of said chamber on rotation of the mold below a predetermined speed.

49. A rotary casting apparatus according to claim 46, in which such spraying means includes a spiral conduit in the chamber.

50. In the art of rotary casting, the method of supervising the rate at which the rotary mold absorbs heat from a charge of ferrous molten metal supplied thereto from a casting therein, which involves introducing said charge into the mold after the mold has

been suitably heated up to a temperature sufficient to insure that said charge following said introduction will distribute itself properly in the mold due to centrifugal force to form the desired casting, then holding in a chamber close to the mold a vapor at a temperature and pressure sufficient to permit the casting to set with that degree of slowness down to a critical temperature point required to insure that the casting after being thus cooled down to said point may thereafter be cooled at a faster rate than before yet without the creation finally of a chilled casting, and then injecting liquid into said chamber at a temperature to be 15 vaporized by the mold temperature and thereby to utilize the latent heat of vaporization principle to abstract heat units quickly from the mold and hence from the casting in the latter, thereby in turn, for speed production purposes, to hasten the reaching by the casting of a sufficient rigidity to permit safe extraction of the casting from the mold. 20

Signed at New York in the county of New York and State of New York this 19th day 25 of December, A. D. 1925.

R. BURDETTE DALE.